

May 28, 1963

E. O. RHODES

3,091,543

PAVING COMPOSITIONS AND METHODS OF MAKING THE SAME

Filed July 23, 1959



INVENTOR.

EDMUND O. RHODES

BY *Raymond P. Wallace*

AGENT

1

3,091,543

## PAVING COMPOSITIONS AND METHODS OF MAKING THE SAME

Edmund O. Rhodes, Pittsburgh, Pa., assignor to Curtiss-Wright Corporation, a corporation of Delaware  
Filed July 23, 1959, Ser. No. 829,041  
4 Claims. (Cl. 106—279)

This invention relates to improved paving structures, and more particularly to bituminous compositions for use in their construction.

As is commonly known, asphalt cements are widely used as binders in the construction of highway surfaces, airport surfaces, and other types of pavement, whether these surfaces are produced by the plant-mix or penetration-macadam procedures. Also used for such purposes, but to a lesser extent, are the standard grades of coal tar designated as RT-11 and RT-12 by the American Society for Testing Materials and the American Association of State Highway Officials.

Each of the two types of binder, namely asphalt cements and road tars, has certain advantages and disadvantages not possessed by the other that are attributable mainly to inherent differences in the raw materials from which they are produced, that is, asphalt from petroleum and road tars from coal tar.

Asphalt cements are better adapted to the present operating conditions at most hot-mix plants, where the mixing temperatures of aggregates and cements range between 275° F. and 325° F. and the temperatures of the mixes at time of laying are usually within a range of 225° F. to 325° F.

On the other hand, owing to the vaporization of volatile components of such coal tar cements as RT-11 and RT-12 at higher temperatures, the preferred temperature range for them is approximately 175° F. to 250° F. and the temperatures of aggregates and fillers to which they are added should not exceed 225° F. Because of these lower required aggregate and binder temperatures, the substitution of coal tar cements for asphalts in hot-mix plants results in lower drying and mixing capacities.

An advantage under service conditions of asphalt cements over coal tar cements of the prior art is a superior viscosity-temperature relationship, more commonly referred to as "temperature-susceptibility." The greater change in consistency with change in temperature that takes place in a typical coal tar cement as contrasted with a typical asphalt cement is illustrated by the data in Table I. In this table are compared the consistencies of the two cements of the prior art, as measured by the "Standard Method of Test for Penetration of Bituminous Materials," ASTM test D5-52. In accordance with this test a standard needle bearing a load of 50 grams was placed with the point in contact with the material and allowed to penetrate for 5 seconds, with the material first at 25° C. and then at 32° C., and the depth of penetration in hundredths of a centimeter was observed.

TABLE I

|                      | Softening point, °C. | Penetration at— |        | Total increase | Increase per °C. |
|----------------------|----------------------|-----------------|--------|----------------|------------------|
|                      |                      | 25° C.          | 32° C. |                |                  |
| Coal tar cement..... | 33                   | 198             | 380    | 182            | 26.0             |
| Asphalt cement.....  | 50.1                 | 50              | 93     | 43             | 6.1              |

It will be observed that the increase in penetration with rise in temperature was much greater for the coal tar cement than for the asphalt cement. To offset the lower softening points of tar cements and their greater tendency to soften under service conditions with rise in tempera-

2

ture, it has been customary to use more densely graded aggregates in the construction of tar concrete and penetration-macadam tar pavements, in order to obtain stabilities comparable with those of asphaltic concretes and asphalt penetration-macadams having somewhat more open aggregate gradings. This necessitates the use of more filler, and more accurate proportioning of the aggregate, filler, and binder when using coal tar cements.

Contrasted with the above disadvantages resulting from the use of coal tar cements in paving structures, however, laboratory and service comparisons have proved that properly constructed paving structures employing tar cements are superior in several important respects to paving structures employing asphalt cements.

Tar cements adhere more strongly to most aggregates, and deteriorate less on contact with or immersion in water for prolonged periods of time; they are much less soluble in jet fuels, gasoline, lubricating oils, fuel oils, and other petroleum distillates and residuals; they impart greater and more permanent skid resistance to pavements in which they are incorporated, and show a greater tendency to "self-heal" if cracking of such pavements occurs.

It is therefore a primary object of this invention to provide a binder material for paving which has the desirable attributes of both the asphalt and coal tar cements of the prior art.

It is another object of the present invention to provide a binder suitable for use under the currently practiced mixing conditions and at the usual operating temperatures.

It is also a principal object of this invention to provide improved binders that will have temperature-susceptibilities superior to those of coal tar cements and comparable to those of asphalt cements.

A further object is the provision of a binder material suitable for the gradations of aggregate generally used in hot-mixes and penetration-macadams.

Another object is to provide a binder capable of maintaining continued strong adhesion to aggregates.

Still a further object of the invention is the provision of a binder composition less subject to deterioration on prolonged contact with or immersion in water.

Yet another object is to provide a binder having minimum solubility in petroleum distillates and residuals.

A further object of the present invention is the provision of a highly skid-resistant paving structure.

Still another object is to provide a paving having self-healing quality.

The foregoing objects and advantages of the invention, and others ancillary thereto, will be readily understood on reading the following specification in connection with the accompanying drawing, in which is shown a fragmentary cross-section in elevation of a paving structure fabricated according to the invention.

In making a binder possessing the advantages enumerated above, bituminous coal is dissolved or colloidally dispersed in coal tar, or in a mixture of coal tar and coal tar oil, in accordance with a process similar to that disclosed in U.S. Patent No. 1,925,005, issued August 29, 1933, to Harold J. Rose and William H. Hill, on a process for making a homogeneous product lower in ash and sulfur content than raw coal.

However, in the present invention the process is carried out in such a manner as to produce binders particularly adapted for use in the construction of highway and airport surfaces of the bituminous concrete type, and surfaces similar to the sheet-asphalt and penetration-macadam types of the prior art. More specifically, coal is digested in coal tar, or in a mixture of coal tar and coal tar oil, in order to produce a digestion product having a temperature-susceptibility superior to that of coal tar alone, or that of a simple mixture of tar and oil. The latter materials are distilled, either before or during the digestion

of the coal, to remove volatile constituents which would evaporate excessively during the hot-mixing operation or from the finished pavement. The precise state of the coal in the digestion product, whether a true solution or a colloidal dispersion, is not known, and it will be understood that the two terms as used herein are intended to be synonymous.

The following examples illustrate some of the ways in which the invention has been carried out.

*Example I*

Distilled coke-oven coal tar, having a softening point of 33° C. and conforming with all the requirements of ASTM Specification D490-47 for grade RT-12, in the proportion of 89.2% by weight was mixed at room temperature with 10.8% of finely ground bituminous coal having the following proximate analysis: moisture 0.48%, volatile material 23.14%, fixed carbon 61.41%, ash 14.97%; the sulfur content was 5.16%.

This mixture was heated in an autoclave with the vent open (no pressure) and with agitation, to remove water and low-boiling distillates. When the temperature reached 400° F. the vent was closed, and heating was continued until the temperature of the mixture reached 600° F. The temperature was then maintained between 600° F. and 620° F. for one hour, during which time the pressure in the autoclave was approximately 20 p.s.i. Heating was then discontinued, the autoclave was cooled until the temperature of the charge had dropped to 400° F., the vent was opened, and the finished binder was drained into a receiver.

*Example II*

The coal used in Example I, in the proportion of 11.4% by weight, was mixed at room temperature with 64.4% of coke-oven coal tar pitch having a softening point of 45° C. and 24.2% of high-boiling coal tar oil having a distillation residue at 355° C. of approximately 75%.

This mixture was charged into the autoclave, heated to 600° F. and held at approximately that temperature for one hour with the vent of the autoclave open (no pressure). After cooling to 400° F. the finished binder was withdrawn from the autoclave.

*Example III*

Crude low-temperature tar made from bituminous coal was heated to 598° F. in the autoclave with the vent open to remove 25.9% of distillate. The residual pitch, with a softening point of approximately 32° C., was mixed at room temperature in the proportion of 64.4% with 24.2% of high-boiling coal tar oil like that used in Example II, and 11.4% of coal like that used in Examples I and II.

This mixture was heated in the autoclave to 400° F. with the vent open, and then to 600° F. with the vent closed. The temperature was maintained at 600° F. for an additional hour with the vent closed; the maximum pressure developed during this period was approximately 40 p.s.i. The mixture was then cooled to 400° F., the vent opened, and the finished binder discharged.

*Example IV*

Crude low-temperature tar was mixed at room temperature with bituminous coal in the proportion of 96% tar to 4% coal. The coal used in this case was not finely ground as in the preceding examples, but had a particle size ranging from  $\frac{3}{8}$ " down to No. 10 screen size. Its approximate analysis was as follows: moisture 0.81%, volatile matter 23.61%, fixed carbon 68.09%, ash 7.49%; its sulfur content was 1.27%.

This mixture was heated to 569° F. in the autoclave with the vent open to a condenser which recovered distillate amounting to 20.2% of total weight. The vent was then closed and heating was continued, maintaining the temperature of the charge at approximately 600° F. for one hour. After cooling to 400° F. the finished binder,

amounting to 73.6% by weight of the original charge, was drained from the autoclave.

In order to compare the four coal digestion binders of the present invention, made as described above, with a typical asphaltic, hot-mix binder and with a representative tar binder of the prior art, each of the six binders are subjected to the following tests.

SOFTENING POINT, RING-AND-BALL METHOD,  
ASTM D36-26

10 A brass ring of  $\frac{5}{8}$ " internal diameter and  $\frac{1}{4}$ " depth is filled with the molten material to be tested. After cooling in water at 5° C. (41° F.) for 15 minutes, a  $\frac{3}{8}$ " steel ball is placed in the center of the upper surface of the sample. The ring containing the sample is then suspended 1" above the bottom of a beaker containing freshly boiled distilled water at 5° C. and 2" below the surface of the water. Heat is applied in such a manner as to raise the temperature of the water by 5° C. each minute. The temperature of the water at the instant when the bituminous material touches the bottom of the vessel is reported as the softening point.

SPECIFIC GRAVITY AT 25° C., ASTM METHOD D71-52

25 By means of a specific gravity balance a  $\frac{1}{2}$ " cube specimen of the binder was weighed in water and in air at 25° C. The specific gravity of the binder was then calculated as follows:

$$30 \text{ Specific gravity} = \frac{\text{Wt. of sample in air}}{\text{Wt. in air} - \text{wt. in water}}$$

PENETRATION AT 25° C. AND 32° C., ASTM METHOD D5-52

35 The depth in hundredths of a centimeter to which a standard needle 2" long and 1.0 to 1.02 mm. in diameter penetrated into a sample of the binder at 25° C. and also at 32° C. was determined. Increase in penetration per degree centigrade between 25° C. and 32° C. was computed as follows:

40 Penetration increase per ° C.

$$\frac{\text{Pen.} @ 32^\circ \text{ C.} - \text{Pen.} @ 25^\circ \text{ C.}}{7}$$

STRIPPING OF BINDER FROM AGGREGATE IN WATER

45 In this test 50 grams of a mixture containing 98% by weight of 20-30 mesh Ottawa sand and 2% of the binder to be tested was agitated vigorously for 15 minutes in water heated to 140° F. The mixture of water and sample was then transferred to a 20-mesh sieve and uncoated (stripped) sand particles were washed through the sieve and into a pan by means of a stream of water heated to approximately 140° F. After decantation of the water from the uncoated particles the latter were dried in the pan and weighed. By multiplying the weight by 2 (since the original weight of the sample was 50 grams), the percentage of stripped particles was determined.

SOLUBILITY IN JET FUEL (JP-4)

50 Jet fuel (JP-4) in the amount of 100 ml. was added to 100 grams of a mixture containing 98% of 20-30 mesh Ottawa sand and 2% of the binder to be tested. The flask containing the above materials were placed in an automatic shaker and agitated vigorously for 15 minutes. The JP-4 was then decanted from the sand-binder mixture and the latter was washed with two 50 ml. portions of fresh JP-4. One-fifth (40 ml.) of the total JP-4 solution was then withdrawn by means of a pipette and transferred to shallow dishes for partial evaporation on a water bath. Evaporation was then continued in an oven to substantially constant weight. The latter multiplied by 5 and divided by 2 (grams of binder in the mixture) gave the percent of binder dissolved by the jet fuel.

MARSHALL STABILITY AND FLOW DETERMINATION

55 A graded limestone aggregate with approximately 7%

passing through a #200 sieve and 100% passing through a  $\frac{3}{8}$ " sieve was mixed at about 300° F. with the optimum proportion of binder as determined by previous tests. Briquets of 4" diameter and approximately 2 $\frac{1}{2}$ " high were made in a mold from the mixture, using 50 blows of the standard Marshall compaction hammer on each end of the specimen. The briquets were allowed to cure in air for at least 24 hours. They were then immersed for 25 minutes in a water bath at 140° F. and tested immediately with a Marshall test assembly in an Instron testing machine. Maximum load (stability) and deformation (flow) at the time of failure were recorded.

CHANGE IN STABILITY AFTER WATER IMMERSION,  
ASTM D1075-54

Graded limestone aggregate passing  $\frac{3}{8}$ " sieve and retained on a #10 sieve was mixed with 4% of each binder. Briquets of 4" diameter and 2 $\frac{1}{2}$ " height were then made from the mixture using Marshall test equipment. Temperatures of aggregate and binder at the time of mixing were about 300° F. and the number of blows with the standard tamper was 50 on each end of each briquet. After atmospheric cooling for at least 8 hours the briquets were immersed in water at 120° F. for four days. They were then placed in water at 140° F. for 25 minutes and tested immediately in the Marshall assembly with Instron equipment to provide the compression.

FLOW TEST AT ATMOSPHERIC TEMPERATURE

Using a mold of the type prescribed by ASTM Method D61-38 (Softening Point of Tar Products, Cube-in-Water Method),  $\frac{1}{2}$ " cubes were prepared from each of the six binders. The six cubes were then placed at the top of a stainless steel plate inclined 30° from the horizontal. The temperature of the room in which the test assembly was placed varied from 26° C. to 28° C. (78.8° F. to 82.4° F.). The way in which each cube deformed and flowed downwardly on the inclined plate was observed and measured after 4 hours, 16 $\frac{1}{2}$  hours, and 22 $\frac{1}{2}$  hours.

Analytical data resulting from the application of the tests described above to each of the six binders are presented in Table II.

TABLE II

|                                                                              | Asphalt Binder | Coal-Tar Binder | Binders Made By Coal Digestion Processes |       |       |       |
|------------------------------------------------------------------------------|----------------|-----------------|------------------------------------------|-------|-------|-------|
|                                                                              |                |                 | I                                        | II    | III   | IV    |
| Softening Point, ° C, R & B-----                                             | 51.8           | 33.0            | 50.8                                     | 45.5  | 49.0  | 48.5  |
| Sp. Gravity at 25° C-----                                                    | 1.030          | 1.200           | 1.255                                    | 1.242 | 1.225 | 1.183 |
| Pen. Increase per ° C. (25°-32° C.), 1/100 cm-----                           | 6.1            | 26.0            | 4.7                                      | 6.8   | 7.1   | 6.1   |
| Percent Stripping in water at 140° F-----                                    | 63.8           | 0.4             | 24.8                                     | 3.4   | 4.0   | 26.0  |
| Marshall Stability at opt. (lbs.)-----                                       | 2326           | 1744            | 3350                                     | 3344  | 3490  | 3612  |
| Marshall Flow at opt. (1/100")-----                                          | 17.4           | 7.7             | 11                                       | 8.5   | 6.0   |       |
| JP-4 Solubility (percent of binder)-----                                     | 97.1           | 11.6            | 16.0                                     | 17.0  | 22.3  |       |
| Change in Stability after Water Immersion, 96 hrs.,<br>120° F., percent----- | -17            | +14.3           | +9.0                                     | +88   | 0     | -2    |
| Flow down 30° Incline, 26-28° Inches After 4 hours-----                      | 1.06           | 2.19            | 0.94                                     | 1.18  | 1.12  | 0.88  |
| Flow down 30° Incline, 26-28° Inches After 16 $\frac{1}{2}$ hours-----       | 1.25           | 3.13            | 0.94                                     | 1.31  | 1.25  | 0.94  |
| Flow down 30° Incline, 26-28° Inches After 22 $\frac{1}{2}$ hours-----       | 1.31           | 3.38            | 0.94                                     | 1.37  | 1.31  | 1.00  |

The data compared are from a typical asphalt binder and a typical coal tar binder of the prior art, and from coal digestion binders made according to Examples I, II, III and IV as discussed hereinabove.

It will be observed that all the binders typifying the present invention have softening points in the neighborhood of that of a typical asphalt cement and much higher than that of a typical coal tar cement. The undesirably low softening points of the usual coal tar cements cause pavements constructed with them to shove and rut excessively unless special precautions are taken in the selection of aggregate gradations and use of increased filler contents. Pavements constructed with binders of the present invention will be less critical with respect to filler content and will be more resistant to rutting or shoving than pavements made with asphalt cements or ordinary coal tar binders.

Specific gravities of binders made in accordance with this invention are appreciably higher than those of asphalt cements and somewhat higher than those of tar cements made in the usual manner. Binders of low specific gravities which, in the case of asphalt cements approach the specific gravity of water, have a greater tendency to float or bleed to the surfaces of pavements in which they are employed and lead to the formation of surfaces that are dangerously slippery when wet.

10 The superior temperature susceptibilities of binders made in accordance with the present invention is shown by their penetration increases per degree rise in temperature between 25° C. and 32° C. They are all much lower than that of the typical coal tar binder and approximately

15 the same as that of the typical asphalt cement. The ability of the present invention to produce pavement binders that will soften less at elevated temperatures and become less hard and brittle at lower temperatures is shown by these comparisons.

20 The binders of the present invention do not show the high tendency of asphalt binders to separate from aggregates on prolonged contact with or immersion in water. Stripping of the sort which results from such separation results in the early destruction of pavements and is highly undesirable.

25 As indicated by Marshall stabilities, the load bearing capacities of pavements made with binders produced in accordance with the present invention are much higher than those of pavements containing asphalt cements or coal tar binders of the prior art.

30 Superior resistance to deformation resulting from abnormally high wheel loadings and channelized traffic is indicated by the low Marshall flow values of the coal digestion binders typifying the present invention.

35 Binders made by the present invention have much lower solubilities than asphalt cements in petroleum distillates or residuals in general and jet fuels, such as JP-4, in particular. The importance of this difference especially on airport surfaces where jet fuel spillage leads to the early destruction of asphalt pavements is readily apparent.

40 Further confirmation of the greater destructive effect

60 of water on asphalt pavements as compared with pavements made with coal digestion binders is furnished by the data for changes in stabilities of briquets immersed in water for 96 hours at 120° F. Briquets containing the typical asphalt cement showed an appreciable decrease in stability whereas some of the briquets made with binders typifying the present invention increased materially in this respect and others showed little or no change.

65 Due to their lower softening points and greater temperature susceptibilities, coal tar cements of the present invention exhibit much greater flow tendencies than typical asphalt paving cements. Self-healing resulting from such coldflow is desirable but too much coldflow can result in low stabilities and excessive deformation under high wheel loadings. By means of the coal digestion process, that is the subject of this invention, it is possible

to control coldflow so as to approximate or duplicate that of asphalt cements if desired.

It is therefore apparent from a consideration of the data in Table II that the binders made by the present invention preserve the desirable characteristics of both the asphalt and the tar of the prior art, in some cases even improving on both.

Referring now to the drawing, there is shown a fragmentary elevation in cross-section of a paving structure incorporating the binder material of the invention. The subgrade 11 is excavated to a depth suitable for the class of road to be built. On the subgrade is laid a base course 12 comprising coarse aggregate and suitable filler material disposed in the interstices thereof. A binder course 13, comprising aggregate of particle size from about one inch down to five percent passing a 200-mesh sieve, hot-mixed with about 4% to 7% of any of the binders made in accordance with the present invention, is laid on the base course and compacted by rolling. Lastly, there is laid a surface or weaving course 14, comprising aggregate having a particle size from one-half inch down to dust, hot-mixed with about 4% to 8% of one of the present binders, and compacted by rolling to a firm, tightly sealed surface. The edges of the road are finished off by a berm 15.

It will be understood that various changes and modifications may be made without departing from the scope of the invention, and it is intended to cover such modifications in the appended claims.

What is claimed is:

1. A method of making paving cement, comprising in combination the steps of mixing at room temperature approximately 90% of distilled coke-oven tar having a softening point of 33° C. with approximately 10% of finely ground bituminous coal, heating said mixture in an autoclave without pressure to approximately 400° F. to remove water and low-boiling distillates, then heating said mixture under approximately 20 p.s.i. pressure to approximately 600° F., maintaining said mixture under said pressure at a temperature between 600° F. and 620° F. for approximately one hour to fully digest said coal in said tar and to form a homogeneous composition thereof, cooling said composition to approximately 400° F., releasing said pressure, and recovering the digestion product.

2. A method of making paving cement, comprising in combination the steps of mixing at room temperature approximately 65% of coke-oven coal tar pitch having a softening point of 45° C. with approximately 11% of finely ground bituminous coal and approximately 24% of high-boiling coal tar oil having a distillation residue

at 355° C. of approximately 75%, heating said mixture to about 600° F. and maintaining said mixture at approximately 600° F. for approximately one hour to fully digest said coal in said pitch and said oil and to form a homogeneous composition thereof.

3. A method of making paving cement comprising in combination the steps of heating low-temperature tar from bituminous coal to approximately 600° F. to remove distillate in the amount of about 26% of the starting weight and to leave a residual pitch with a softening point of approximately 32° C., cooling said pitch, mixing said pitch at room temperature in the proportion of approximately 65% with approximately 24% of high-boiling coal tar oil and approximately 11% of finely ground bituminous coal, heating said mixture in an autoclave without pressure to approximately 400° F. to distill off volatile components, then heating said mixture to approximately 600° F. under approximately 40 p.s.i. pressure maintaining said mixture at about 600° F. under said pressure for approximately one hour to fully digest said coal in said pitch and said oil and to form a homogeneous composition thereof, cooling said composition to approximately 400° F., releasing said pressure, and recovering the digestion product.

4. A method of making paving cement, comprising in combination the steps of mixing approximately 96% of low-temperature coal tar at room temperature with approximately 4% of crushed bituminous coal having particle sizes ranging from No. 10 screen size to  $\frac{3}{8}$ ", heating said mixture in an autoclave to a temperature in the neighborhood of 600° F. without pressure to distill off volatile components in the amount of approximately 20% by weight of the original mixture, and maintaining the residual mixture at approximately 600° F. under approximately 20 p.s.i. pressure for about one hour to fully digest said coal in said tar and to form a homogeneous composition thereof.

#### References Cited in the file of this patent

| UNITED STATES PATENTS |                |               |
|-----------------------|----------------|---------------|
| Re. 9,207             | Bailey         | May 18, 1880  |
| 875,196               | Lovejoy        | Dec. 31, 1907 |
| 1,500,451             | Hacker         | July 8, 1924  |
| 45 2,629,669          | Anderton       | Feb. 24, 1953 |
| 2,861,895             | Hardman        | Nov. 25, 1958 |
| 2,888,357             | Pittman et al. | May 26, 1959  |

#### FOREIGN PATENTS

|    |         |               |               |
|----|---------|---------------|---------------|
| 50 | 334,336 | Great Britain | Sept. 4, 1930 |
|----|---------|---------------|---------------|